



US005964907A

**United States Patent** [19]**Farmer et al.****Patent Number:** **5,964,907****Date of Patent:** **Oct. 12, 1999**[54] **FUEL COMPOSITIONS CONTAINING ESTERAMINES**

[75] Inventors: **Robert F. Farmer**, Barrington, Ill.; **Ralph Franklin**, Danbury, Conn.; **Michael Kanakia**, New Fairfield, Conn.; **James F. Gadberry**, Danbury, Conn.

[73] Assignee: **Akzo Nobel N.V.**, Arnhem, Netherlands

[21] Appl. No.: **08/698,206**

[22] Filed: **Aug. 14, 1996**

[51] **Int. Cl.<sup>6</sup>** ..... **C10L 1/18**; C10L 1/22

[52] **U.S. Cl.** ..... **44/391**; **44/399**

[58] **Field of Search** ..... **44/391, 399**

[56] **References Cited**

## U.S. PATENT DOCUMENTS

|           |         |                   |       |        |
|-----------|---------|-------------------|-------|--------|
| 2,110,274 | 3/1938  | Mikeska et al.    | ..... | 44/391 |
| 2,854,323 | 9/1958  | Shen et al.       | .     |        |
| 3,063,819 | 11/1962 | Watt et al.       | .     |        |
| 3,091,521 | 5/1963  | Liao              | ..... | 44/399 |
| 3,117,931 | 1/1964  | Westlund et al.   | .     |        |
| 3,183,070 | 5/1965  | Udelhofen         | ..... | 44/391 |
| 3,240,575 | 3/1966  | Miller et al.     | .     |        |
| 3,381,022 | 4/1968  | Le Suer           | .     |        |
| 3,658,707 | 4/1972  | Delafield et al.  | .     |        |
| 3,676,483 | 7/1972  | Hu                | .     |        |
| 3,807,973 | 4/1974  | Iwama et al.      | .     |        |
| 3,890,357 | 6/1975  | Rubin et al.      | .     |        |
| 3,920,729 | 11/1975 | Sagawa et al.     | ..... | 44/399 |
| 3,957,854 | 5/1976  | Miller            | .     |        |
| 4,002,569 | 1/1977  | Rubin et al.      | .     |        |
| 4,204,481 | 5/1980  | Malec             | ..... | 44/391 |
| 4,234,435 | 11/1980 | Meinhardt et al.  | .     |        |
| 4,622,047 | 11/1986 | Bernasconi et al. | .     |        |
| 4,639,256 | 1/1987  | Axelrod et al.    | ..... | 44/399 |
| 4,670,021 | 6/1987  | Nelson et al.     | ..... | 44/399 |

|           |        |                  |       |
|-----------|--------|------------------|-------|
| 4,810,263 | 3/1989 | Zimmerman et al. | .     |
| 5,194,068 | 3/1993 | Mohr et al.      | ..... |
| 5,298,038 | 3/1994 | Hashimoto et al. | ..... |
| 5,407,452 | 4/1995 | Cherpeck         | .     |
| 5,597,390 | 1/1997 | Loper            | ..... |

## FOREIGN PATENT DOCUMENTS

|             |         |                    |   |
|-------------|---------|--------------------|---|
| 650405      | 11/1964 | Belgium            | . |
| 0085803     | 8/1983  | European Pat. Off. | . |
| 0117108     | 3/1984  | European Pat. Off. | . |
| 0353713     | 2/1990  | European Pat. Off. | . |
| 0464489     | 1/1992  | European Pat. Off. | . |
| 1211144     | 3/1960  | France             | . |
| 2576032     | 7/1986  | France             | . |
| 2144199     | 3/1973  | Germany            | . |
| 2559480     | 1/1977  | Germany            | . |
| 57-170993   | 10/1982 | Japan              | . |
| 59-189192   | 10/1984 | Japan              | . |
| 60-137998   | 7/1985  | Japan              | . |
| 60-166389   | 8/1985  | Japan              | . |
| 61-281198   | 12/1986 | Japan              | . |
| 62-109893   | 5/1987  | Japan              | . |
| 899261      | 6/1962  | United Kingdom     | . |
| 1062605     | 3/1967  | United Kingdom     | . |
| 1410788     | 10/1975 | United Kingdom     | . |
| WO 9303120  | 2/1993  | WIPO               | . |
| WO 96/34177 | 10/1996 | WIPO               | . |

## OTHER PUBLICATIONS

Owen, "Gasoline and Diesel Fuel Additives", *Critical Reports on Applied Chemistry*, vol. 25, pp. 23-33, date unavailable.

*Primary Examiner*—Jacqueline V. Howard  
*Attorney, Agent, or Firm*—Dilworth & Barrese

[57]

## ABSTRACT

Engine deposits are reduced by adding an effective deposit-controlling amount of an esteramine to hydrocarbon fuel.

**27 Claims, 2 Drawing Sheets**



**Fig. 1**

**Fig. 2**

## 1

FUEL COMPOSITIONS CONTAINING  
ESTERAMINES

## BACKGROUND

## 1. Technical Field

This disclosure relates to fuel compositions containing deposit control additives and methods for reducing deposits on the surface of engine components and within the combustion chamber. More specifically, this disclosure relates to fuel compositions containing a deposit-controlling amount of esteramines to inhibit and control engine deposits.

## 2. Background of Related Art

It is well known that automobile engines tend to form deposits within the combustion chamber and on the surface of engine components, such as carburetor ports, throttle bodies, fuel injectors, intake ports, intake valves, piston tops, and cylinder heads due to the evaporation, oxidation and polymerization of hydrocarbon fuel. These deposits, even when present in relatively minor amounts, often cause noticeable driveability problems, such as stalling and poor acceleration. Moreover, engine deposits can significantly increase an automobile's fuel consumption and production of exhaust pollutants. Therefore, the development of effective fuel detergents or "deposit control" additives to prevent or control such deposits is of considerable importance.

It has now been discovered that certain esteramines are surprisingly useful for reducing engine deposits when employed as fuel additives in fuel compositions.

## SUMMARY

Novel fuel compositions described herein comprise a major amount of fuel and an effective deposit-controlling amount of at least one esteramine of the general formula:



wherein  $R^1$  is a  $C_7-C_{21}$  hydrocarbon group, preferably a  $C_7-C_{21}$  saturated or unsaturated alkyl group;  $x$  is 1, 2 or 3;  $y$  and  $z$  are individually selected from 0, 1 or 2;  $x+y+z=3$ ;  $R^2$  is selected from the group consisting of  $C_1-C_6$  alkylene groups and  $-(R^5O)_nR^5-$  groups wherein each  $R^5$  can be the same or different and is independently selected from the group consisting of linear or branched  $C_1-C_6$  alkylene groups and  $n$  is 1 to 60,  $R^3$  and  $R^4$  can be the same or different and are individually selected from the group consisting of  $C_1-C_6$  alkyl groups,  $-(R^5O)_nH$  groups wherein  $R^5$  and  $n$  are as defined above, and  $-R^6-N-R^7R^8$  groups wherein  $R^6$  is a  $C_1$  to  $C_6$  linear or branched alkylene group, and  $R^7$  and  $R^8$  can be the same or different and are individually selected from the group consisting of  $R^3$ ,  $R^4$  and



groups wherein  $R^1$ ,  $R^2$ ,  $R^3$ , and  $R^4$  are as defined above.

In particularly useful embodiments, the esteramine is prepared by reacting a fatty acid with an alkanolamine, a polyalkanolamine, an alkoxyLATED amine or an alkoxyLATED polyamine. The esteramine can be a mono-, di-, tri- or tetra-ester and can be used alone or with other deposit-control additives. In a particularly useful embodiment, the

## 2

presently disclosed esteramine additives are used in combination with a known polyetheramine additive. The resulting combination of additives surprisingly provides a synergistic effect with respect to reducing engine deposits.

5 Methods for reducing engine deposits in an internal combustion engine are also described. The methods comprise operating an engine with a fuel comprising an effective deposit-controlling amount of an esteramine; preferably an esteramine prepared by reacting a fatty acid with an alkanolamine or an alkoxyLATED amine.

## BRIEF DESCRIPTIONS OF THE DRAWINGS

Various embodiments are described herein with reference to the drawings wherein:

15 FIG. 1 is a graph depicting measured engine intake valve deposits resulting from 80 hour operation of a four cycle engine using fuel containing various additive compositions, including presently described esteramine deposit control additive compositions; and

20 FIG. 2 is a graph depicting measured engine deposits resulting from 80 hour operation of four cycle engine using fuel containing various additive compositions, including presently described esteramine deposit control additive compositions and showing the synergistic effects obtained when the presently described deposit control additives are combined with a known polyetheramine additive.

DETAILED DESCRIPTION OF PREFERRED  
EMBODIMENTS

30 The fuel compositions described herein contain a major amount of gasoline and an effective deposit-controlling amount of at least one esteramine. The esteramine is of the general formula:



40 wherein  $R^1$  is a  $C_7-C_{21}$  hydrocarbon group, preferably a  $C_7-C_{21}$  saturated or unsaturated alkyl group;  $x$  is 1, 2 or 3;  $y$  and  $z$  are individually selected from 0, 1 or 2;  $x+y+z=3$ ;  $R^2$  is selected from the group consisting of  $C_1-C_6$  alkylene groups and,  $-(R^5O)_nR^5-$  groups wherein each  $R^5$  can be the same or different and is independently selected from the group consisting of linear or branched  $C_1-C_6$  alkylene group and  $n$  is 1 to 60,  $R^3$  and  $R^4$  can be the same or different and are individually selected from the group consisting of  $C_1-C_6$  alkyl groups,  $-(R^5O)_nH$  groups wherein  $R^5$  and  $n$  are as defined above, and  $-R^6-N-R^7R^8$  groups wherein  $R^6$  is a  $C_1$  to  $C_6$  linear or branched alkylene group, and  $R^7$  and  $R^8$  can be the same or different and are individually selected from the group consisting of  $R^3$ ,  $R^4$  and



55 60 groups wherein  $R^1$ ,  $R^2$ ,  $R^3$ , and  $R^4$  are as defined above.

In particularly useful embodiments, the esteramine is prepared by reacting a fatty acid with an alkanolamine, a polyalkanolamine, an alkoxyLATED amine or alkoxyLATED polyamine. The fatty acid may be hydrogenated and is preferably a saturated fatty acid. Long chain fatty acids having 12 carbon atoms or more are particularly preferred for use in making the esteramine. Most preferred are long

chain fatty acids having 16 to 18 carbon atoms, i.e., the tallow acids, including hydrogenated and partially hydrogenated tallow.

The fatty acid is reacted with an alkanolamine to provide an esteramine. Amines having one, two or three active sites can be employed to produce mono-, di-, or triesters, respectively. Thus, for example, triethanol amine can be reacted with a fatty acid to provide a triester. Methyldiethanolamine will produce a diester when reacted with the fatty acid. Dimethylethanolamine will react with a fatty acid to generate a monoester. The conditions under which amines can be reacted with fatty acids to produce the present esteramines are known to those skilled in the art. Such reaction conditions are disclosed, for example, in PCT Publication No. WO91/01295, the disclosure of which is incorporated herein by this reference.

It is also possible to employ an alkoxylated amine or alkoxylated polyamine in preparing the present esteramine additives. Thus, for example, amines having one or more  $(R^5O)_nH$  groups wherein  $R^5$  and  $n$  are as mentioned above can be used as a starting material to produce the present esteramine deposit control additives. Such alkoxylated amines are available, for example, under the names Propomeen® and Ethorneen® from Akzo Nobel Chemicals Inc., Chicago, Ill. Preferably  $R^5$  is selected from ethylene, propylene and mixtures thereof. The conditions under which alkoxylated amines are reacted with fatty acids to produce esteramines are also known and are described, for example, in U.S. Pat. No. 5,523,433, the disclosure of which is incorporated by reference.

It is also possible to synthesize suitable esteramines by reacting a fatty acid with a diamine having at least one alkanol group of the general formula:



wherein  $R^6$  is as mentioned above;  $R$ , which can be the same or different in each instance, is selected from H,  $C_1-C_6$  saturated or unsaturated, substituted or unsubstituted, branched or unbranched alkyl and  $C_1-C_6$  alkanol. Thus, for example, a tetraester can be prepared by reacting a fatty acid with a diamine of the formula:



Other starting materials for forming esteramines using diamines as a starting material will be apparent to those skilled in the art.

Esteramines suitable for use in connection with the fuel compositions and methods described in this disclosure should be soluble in the fuel and should not impart excessive water sensitivity to the fuel. Esteramines useful in the present invention are available from Akzo Nobel Chemicals Inc., Chicago, Ill.

The present fuel compositions contain an effective deposit-controlling amount of esteramine additives. The exact amount of additive that is effective in controlling deposits will depend on a variety of factors including the type of fuel employed, the type of engine and the presence of other fuel additives.

In general, the concentration of the esteramines in hydrocarbon fuel will range from about 50 to about 2500 parts per million (ppm) by weight, preferably from 75 to 1,000 ppm, more preferably from 200 to 500 ppm. When other deposit control additives are present, a lesser amount of the present additive may be used.

The present esteramine additives may also be formulated as a concentrate using an inert stable oleophilic (i.e., dissolves in gasoline) organic solvent boiling in the range of about 150° F. to 400° F. (about 65° C. to 205° C.). Preferably, an aliphatic or an aromatic hydrocarbon solvent is used, such as benzene, toluene, xylene or high-boiling aromatics or aromatic thinners. Aliphatic alcohols containing about 3 to 8 carbon atoms, such as isopropanol, isobutylecarbinol, n-butanol and the like, in combination with hydrocarbon solvents are also suitable for use with the present additives. In the concentrate, the amount of the additive will generally range from about 10 to about 70 weight percent, preferably to 50 weight percent, more preferably from 20 to 40 weight percent.

In gasoline fuels, other fuel additives may be employed with the additives of the present invention, including, for example, oxygenates, such as t-butyl methyl ether, anti-knock agents, such as methylcyclopentadienyl manganese tricarbonyl, and other dispersants/detergents, such as hydrocarbyl amines, hydrocarbyl poly-(oxyalkylene) amines, or succinimides. Additionally, antioxidants, metal deactivators and demulsifiers may be present.

A fuel-soluble, nonvolatile carrier fluid or oil may also be used with the esteramine additives described herein. The carrier fluid is a chemically inert hydrocarbon-soluble liquid vehicle which substantially increases the nonvolatile residue (NVR), or solvent-free liquid fraction of the fuel additive composition while not overwhelmingly contributing to octane requirement increase. The carrier fluid may be a natural or synthetic oil, such as mineral oil, refined petroleum oils, synthetic polyalkanes and alkenes, including hydrogenated and unhydrogenated polyalphaolefins, synthetic polyoxyalkylene-derived oils, esters and polyesters.

The carriers fluids are typically employed in amounts ranging from about 100 to about 5000 ppm by weight of the hydrocarbon fuel, preferably from 400 to 3000 ppm of the fuel. Preferably, the ratio of carrier fluid to deposit control additive will range from about 0.5:1 to about 10:1, more preferably from 1:1 to 4:1, most preferably about 2:1.

When employed in a fuel concentrate, carrier fluids will generally be present in amounts ranging from about 20 to about 60 weight percent, preferably from 30 to 50 weight percent.

## EXAMPLES

The following examples are presented to illustrate specific embodiments of the present compositions and methods. These examples should not be interpreted as limitations upon the scope of the invention.

In the following examples, references to Esteramines I-VII relate to the following compounds:

- I. N,N-Dimethylethanolamine cocoate ester
- II. N-Methyldiethanolamine di(hydrogenated tallowate) ester
- III. Triethanolamine tritallowate ester
- IV. N-Methyldiethanolamine ditallowate ester
- V. N,N,N',N'-Tetra(2-hydroxyethyl)-1,3-propanediamine tetralallowate ester
- VI. Alkoxylated methylamine ditallowate ester
- VII. N,N-bis-(2-hydroxyethyl)-3-dimethylaminopropylamine ditallowate ester.

### Examples 1-6

Esteramines I and II were used to formulate six fuel compositions which were tested to evaluate the tendency of the fuel compositions to form deposits on heated metal surfaces.

The compositions were evaluated using an induction system deposit (ISD) apparatus which is a bench-scale analytical laboratory tool that simulates two essential conditions that occur in the gasoline induction systems of spark-ignition engines: high temperature and thin film oxidation of atomized gasoline. In an ISD test, a fuel/air mixture is aspirated onto the outer surface of a internally heated metal deposit tube, in a flat spray pattern. This produces a roughly elliptical deposit on the cylindrical tube surface which can be weighed and visually evaluated. Test results from additized fuels can be interpreted as an indication of the relative effectiveness of the additives at reducing the deposit forming tendency of the fuel in a simulated induction system environment.

Additized samples for the ISD test were prepared by taking appropriate aliquots from 10 g/l stock solutions of the additives in the test fuel. 150 g of each sample was prepared and filtered through a 0.8 micro-meter membrane filter. Immediately after filtration, 150 ml of each test sample was tested on the ISD apparatus. Test data was recorded as deposit weight to nearest 0.1 mg. Tabulated data for additized fuel was presented as the percent of the "baseline" deposit produced by the unadditized test fuel.

$$\% \text{ of Baseline} = \frac{\text{mg deposit (additized fuel)}}{\text{mg deposit (unadditized fuel)}} \times 100$$

The test parameters used for all the tests are as follows:

|                   |                                                                      |
|-------------------|----------------------------------------------------------------------|
| Test Temp.        | 450° F. (232° C.)                                                    |
| Sample Size       | 150 ml                                                               |
| Fuel Flow Rate    | 2 ml/min                                                             |
| Air Flow Rate     | 15 l/min                                                             |
| Cylinder Material | Aluminum                                                             |
| Test Fuel         | Formulated by Phillips Petroleum Co. for port injector fouling tests |

The results which are presented in Table I, show that both esteramine products reduce the fuel deposit weight to between 40% and 45% of the level produced with unadditized fuel when they are used by themselves at 300 ppm by weight in the test fuel. When either product is used in combination with a solvent neutral oil, the deposit reduction is significantly improved (See Examples 3-6 in Table I.)

TABLE I

|                                | Ex. 1 | Ex. 2 | Ex. 3 | Ex. 4 | Ex. 5 | Ex. 6 | Ex. A |
|--------------------------------|-------|-------|-------|-------|-------|-------|-------|
| Esteramine I                   | 300*  | —     | 300   | —     | —     | —     | —     |
| Esteramine II                  | —     | 300   | —     | 300   | 300   | 150   | —     |
| Solvent                        | —     | 300   | 500   | 500   | 500   | 500   | 500   |
| Neutral Oil**                  | 44    | 42    | 27    | 11    | 15    | 28    | 58    |
| ISD Deposit<br>(% of Baseline) |       |       |       |       |       |       |       |

\*Additive Concentration is given as ppm by weight in test fuel.

\*\*The Solvent Neutral Oil used was Kenedex 600, Kenedex/Amali Div. of Witco Corp.

### Examples 7-13

Seven fuel compositions containing esteramine additives were formulated and tested to evaluate the additive's effectiveness at reducing deposits in an operating engine.

The fuel compositions identified in Table II were used to operate pre-cleaned Honda Genset Engines for 80 hours.

The engines were then disassembled and any deposits on the underside of the inlet valves were carefully removed and weighed. Any deposits on the piston top and combustion chamber of these four-cycle engines were also carefully collected and weighed. A baseline was established by operating a Honda Genset Engine using a test fuel containing no additives. The results are reported in Table II and are graphically depicted in FIG. 1.

TABLE II

| Example | Additive       | Combustion Chamber Deposit (g) | Intake Valve Deposit (mg) | Intake Valve Deposit (% of Baseline) |
|---------|----------------|--------------------------------|---------------------------|--------------------------------------|
| CONTROL | NONE           | 1.2                            | 205                       | 100%                                 |
| 7       | Esteramine I   | 0.4                            | 105                       | 51%                                  |
| 8       | Esteramine II  | 1.3                            | 29                        | 14%                                  |
| 9       | Esteramine III | 1.1                            | 49                        | 24%                                  |
| 10      | Esteramine IV  | 0.7                            | 41                        | 20%                                  |
| 11      | Esteramine V   | 1.4                            | 51                        | 25%                                  |
| 12      | Esteramine VI  | 1.2                            | 55                        | 27%                                  |
| 13      | Esteramine VII | 1.4                            | 113                       | 55%                                  |

In each case the concentration of the identified additive was 400 ppm and 500 ppm of a neutral solvent oil was also used.

As is evident from the values reported in Table II, the present esteramine additives reduced intake valve deposits by a minimum of about half to as much as 86% compared to the amount of deposit produced by non-additized fuel.

### Examples 14 and 15

Fuel compositions were prepared by adding 400 ppm of the Esteramine II used in Example 2 to two different commercial fuels; namely Shell 87 octane regular unleaded gas and Exxon 87 octane regular unleaded gas. The chemical make-up of any additive package already in the commercial fuels was unknown. Each fuel composition was used to operate a Honda Genset Engine for 80 hours. Then, any deposits formed in the intake valve and combustion chamber were carefully removed and weighed as previously described. For comparison purposes the commercial fuels were tested without the addition of the present esteramine additives. The results are reported in Table III.

45

| Example No. | Composition                          | Intake Valve Deposit (mg) | Combustion Chamber Deposit (g) |
|-------------|--------------------------------------|---------------------------|--------------------------------|
| Control     | Shell Regular Gas (unleaded)         | 0.0                       | 1.9                            |
| Example 14  | Shell Regular Gas Plus Esteramine I  | 0.0                       | 1.1                            |
| Control     | Exxon Regular Gas (unleaded)         | 38                        | 2.5                            |
| Example 15  | Exxon Regular Gas Plus Esteramine II | 2.5                       | 1.3                            |

As the data in Table III show, the present esteramine additives significantly enhance any deposit control additives contained in the commercially available fuels tested.

### Examples 16 and 17

The unexpected synergistic effects of the present esteramines when combined with a known polyetheramine additive

were shown as follows: An 87 octane base fuel containing no additives was tested in the manner previously described to establish a baseline of deposits at the intake valve and combustion chamber of a four cycle engine. An esteramine deposit control additive in accordance with this disclosure (Esteramine II) was added to the base fuel to a concentration of 300 ppm and tested in the manner previously described to determine the amount of intake valve and combustion chamber deposits generated. A similar fuel composition containing the base fuel and 400 ppm of a polyetheramine additive that is commercially available under the name Techron from Chevron Corp. was also tested. Finally, a fuel composition containing the base fuel, 200 ppm of Esteramine II and 300 ppm polyetheramine was prepared and tested. The results are summarized in Table IV and graphically depicted in FIG. 2.

TABLE IV

| Example No. | Additive Composition              | In the Valve Deposit (mg) | Combustion Chamber Deposit (g) |
|-------------|-----------------------------------|---------------------------|--------------------------------|
| Control     | None                              | 205                       | 1.2                            |
| 16          | Esteramine II                     | 24                        | 1.3                            |
| Control     | Polyetheramine                    | 6.3                       | 2.2                            |
| 17          | Esteramine II plus Polyetheramine | 1.3                       | 1.4                            |

As the data in Table IV and FIG. 2 show, with respect to intake valve deposits the combined effects of the present esteramine additive and known polyether additive is greater than either of the additives individually.

It will be understood that various modifications may be made to the embodiments disclosed herein. Therefore, the above description should not be construed as limiting, but merely as exemplifications of preferred embodiments. Those skilled in the art will envision other modifications within the scope and spirit of the claims appended hereto.

What is claimed is:

1. A method for reducing combustion chamber and intake valve deposits in a four cycle engine, the method comprising:

preparing a four cycle engine fuel composition by combining a major amount of gasoline with an effective intake valve and combustion chamber deposit-controlling amount of an additive, the additive consisting essentially of at least one esteramine of the formula:



wherein  $R^1$  is a hydrocarbon group derived from coco, tallow or hydrogenated tallow fatty acid;  $x$  is 2 or 3;  $y$  and  $z$  are individually selected from 0 or 1;  $x+y+z=3$ ,  $R^2$  is selected from the group consisting of  $C_1-C_6$  alkylene groups and  $-(R^5O)_nR^5-$  groups wherein each  $R^5$  can be the same or different and is independently selected from the group consisting of linear or branched  $C_1-C_6$  alkylene groups and  $n$  is 1 to 60,  $R^3$  and  $R^4$  can be the same or different and are individually selected from the group consisting of  $C_1-C_6$  alkyl groups  $-(R^5O)_nH$  groups wherein  $R^5$  and  $n$  are as defined above, and  $-R^6-N-R^7R^8$  groups wherein  $R^6$  is a  $C_1$  to  $C_6$  linear or branched alkylene group, and  $R^7$  and  $R^8$  can be the same or different and are individually selected from the group consisting of  $R^3$ ,  $R^4$  and  $(R^1-COO-R^2)-$  groups wherein  $R^1$ ,  $R^2$ ,  $R^3$  and  $R^4$  are as defined above.

groups wherein  $R^1$ ,  $R^2$ ,  $R^3$  and  $R^4$  are as defined above; and

operating a four cycle engine using the fuel composition.

2. A method as in claim 1 wherein the esteramine is a diesteramine.

3. A method as in claim 1 wherein the esteramine is a triesteramine.

4. A method as in claim 1 wherein the esteramine is a tetraesterdiamine.

5. A method as in claim 1 wherein esteramine is added to the fuel at a concentration from about 50 to about 2500 ppm.

6. A method as in claim 1 wherein esteramine is added to the fuel at a concentration from about 200 to about 500 ppm.

7. A method as in claim 1 wherein the step of preparing a four cycle engine fuel further comprises adding a polyetheramine to the hydrocarbon fuel.

8. A method for reducing combustion chamber and intake valve deposits in a four cycle engine, comprising:

providing a hydrocarbon fuel for a four cycle engine; and adding to the hydrocarbon fuel an effective combustion chamber and intake valve deposit-controlling amount of an additive, the additive consisting essentially of at least one esteramine of the formula:



30 wherein  $R^1$  is a hydrocarbon group derived from coco, tallow or hydrogenated tallow fatty acid;  $x$  is 2 or 3;  $y$  and  $z$  are individually selected from 0 or 1;  $x+y+z=3$ ,  $R^2$  is selected from the group consisting of  $C_1-C_6$  alkylene groups and  $-(R^5O)_nR^5-$  groups wherein each  $R^5$  can be the same or different and is independently selected from the group consisting of linear or branched  $C_1-C_6$  alkylene groups and  $n$  is 1 to 60,  $R^3$  and  $R^4$  can be the same or different and are individually selected from the group consisting of  $C_1-C_6$  alkyl groups  $-(R^5O)_nH$  groups wherein  $R^5$  and  $n$  are as defined above, and  $-R^6-N-R^7R^8$  groups wherein  $R^6$  is a  $C_1$  to  $C_6$  linear or branched alkylene group, and  $R^7$  and  $R^8$  can be the same or different and are individually selected from the group consisting of  $R^3$ ,  $R^4$  and  $(R^1-COO-R^2)-$  groups wherein  $R^1$ ,  $R^2$ ,  $R^3$  and  $R^4$  are as defined above.

35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 885



**11**

wherein R<sup>1</sup> is a C<sub>7</sub>–C<sub>21</sub> hydrocarbon group; R<sup>2</sup> is selected from the group consisting of C<sub>1</sub>–C<sub>6</sub> alkylene groups and —(R<sup>5</sup>O)<sub>n</sub>R<sup>5</sup>— groups wherein each R<sup>5</sup> can be the same or different and is independently selected from the group consisting of linear or branched C<sub>1</sub>–C<sub>6</sub> alkylene groups and n is 1 to 60 and R<sup>6</sup> is a C<sub>1</sub> to C<sub>6</sub> linear or branched alkylene group; and 5

**12**

R<sup>7</sup> is selected from the group consisting of C<sub>1</sub>–C<sub>6</sub> alkyl groups, —(R<sup>5</sup>O)<sub>n</sub>H groups where R<sup>5</sup> and n are as defined above and (R<sup>1</sup>C(O)OR<sup>2</sup>)— groups where R<sup>1</sup> and R<sup>2</sup> are as defined above.

\* \* \* \* \*